

Jan. 3, 1939.

H. DREYFUS ET AL

2,142,721

MANUFACTURE OF ARTIFICIAL YARNS OR OTHER MATERIALS

Original Filed Feb. 1, 1935



Inventors  
H. Dreyfus  
D. Finlayson  
by  
G. L. Bergman  
Attorneys

## UNITED STATES PATENT OFFICE

2,142,721

MANUFACTURE OF ARTIFICIAL YARNS OR  
OTHER MATERIALS

Henry Dreyfus, London, and Donald Finlayson,  
Spondon, near Derby, England, assignors to  
Celanese Corporation of America, a corporation  
of Delaware

Original application February 1, 1935, Serial No.  
4,511. Divided and this application January  
18, 1937, Serial No. 121,150. In Great Britain  
February 2, 1934

10 Claims. (Cl. 8—132)

This invention relates to new processes for the production of artificial filaments, threads, yarns, ribbons, foils, films, and other materials having a basis of cellulose acetate or other cellulose ester or ether and having improved properties, particularly improved tensile strength. The application is a divisional application of our application S. No. 4,511 filed February 1, 1935.

The production of materials of the above character, and particularly filaments and similar textile materials, having an increased tensile strength is of considerable importance from the commercial point of view. The processes which have been hitherto proposed with this object have involved subjecting the threads or other materials to a stretching operation, and in order to obtain substantial increases in tensile strength it has been considered necessary to subject the materials to the action of liquids which are solvents or swelling agents for the materials, for example dioxane, acetone, acetic acid, and diacetone alcohol, all applied for example in aqueous solution. It has also been suggested to use such liquids in the vapour state.

It has now been discovered that materials having a basis of cellulose acetate or other cellulose ester or ether may have their tensile strength increased in a very simple manner by subjecting them to a stretching operation in hot water under pressure at a temperature above 100° C.

The water may for example be at a temperature of 110°, 120°, 130° C. or higher and at a pressure of, for example, 10, 20, 30 pounds or more per square inch above atmospheric pressure. The best conditions for treatment are dependent upon the degree of stretch required and the rate of stretching and upon a number of factors to be referred to hereinafter. For relatively low degrees of stretch the pressure may be only slightly above atmospheric pressure, for example only a few pounds above atmospheric pressure.

By the new process degrees of stretch of 200% or more may be obtained, particularly when the water is employed at a temperature above 125° C., for example stretches of many hundreds per cent.

By employing appropriate temperatures for giving high degrees of stretch, filaments and threads of very fine denier and similarly thin foils, films and the like may be obtained.

Textile materials to be treated in accordance with the invention may be threads or other materials composed of continuous filaments, or may be spun yarns made of short or more or less long lengths of filament, and may be obtained by cut-

ting up or by any other suitable process, for example the process of U. S. Patent No. 2,077,078. The materials may initially have any desired lustre from a high lustre to medium lustre or approximately the lustre of natural silk or even a dull lustre or no lustre at all. Thus, the materials may have a low lustre due to the presence therein of titanium dioxide or other pigments. Preferably the materials on entering the hot water are substantially free from volatile solvents.

The operation may be carried out on the materials in any suitable form; for example threads may be stretched in hank form, for instance between rollers positioned in a vessel containing the hot water. Preferably, however, stretching of the materials is effected during the course of their travel from one point to another. The treatment may be applied to a single thread, e. g. during winding from a cake or cheese or bobbin on to a bobbin, or it may be applied to a number of threads simultaneously. Thus, artificial threads may be stretched while running from one creel of bobbins to another creel. When simultaneously stretching a number of threads, it is advantageous to arrange the threads in parallel alignment in the form of a sheet or, if desired, in the form of two parallel sheets.

The stretching operation may be carried out so that the desired degree of stretch is obtained in a single stage of stretching or, if desired, intermediate rollers or other stretching devices may be provided so as to carry out the stretch in more than one stage.

Apparatus enabling the stretching to be carried out is described in our co-pending application No. 47,798 filed November 1, 1935. Broadly the apparatus comprises a substantially closed chamber for the hot water provided with heating means for water in the chamber and with one or more inlet and outlet orifices for the materials, associated with means for stretching the materials while in the chamber. The chamber may be provided with a source of supply of water under pressure and means for removing the water continuously. The water chamber may further be provided with a pressure-relief valve, a water drain-off and a pressure gauge. The water chamber is constructed to resist the required pressure and the inlet and outlet orifices for the materials are sufficiently small to enable the pressure to be maintained.

The accompanying drawing illustrates diagrammatically a suitable apparatus for carrying out the stretching with hot water under pressure.

Figure 1 shows a longitudinal view of the ap-

5

10

15

20

25

30

35

40

45

50

55

55

paratus, largely in section, while Figure 2 shows a horizontal cross-section of the hot water chamber.

The threads 1 from a creel of bobbins 2 are carried through nip rollers 3 into the hot water chamber 4, are drawn therethrough by nip rollers 5 and taken up on a creel of bobbins 6. To the hot water chamber 4 are secured closure plates 7 and 8 suitably perforated for the passage of the threads as illustrated in Figure 2. Water enters the chamber 4 by a pipe 9 from a suitable reservoir (not shown) maintained under pressure, for example by means of compressed air, and leaves the chamber by a pipe 10. The chamber 4 is further provided with a pressure gauge 11 and with a steam heating coil 12 for maintaining the desired temperature. Suitable catch trays, illustrated diagrammatically at 13 and 14, provided with drains, serve to catch the water exuded through the orifices in the closure plates 7 and 8. A drain 15 is provided for draining the hot water chamber 4, for example for threading up the apparatus.

The length of thread subjected to the action of the hot water may be quite short and good stretching may be obtained with a length of less than one foot. However, it is preferable to extend the length of the hot water chamber to some feet, for example 3-6 feet or more, the precise length depending upon the temperature and the amount and rate of stretching.

For any particular degree of stretch and rate of stretching, a range of temperatures is available. The best temperature at which to work depends upon a number of factors, including the twist on the initial thread which for quick stretching should be as small as possible, the nature of the cellulose derivative under treatment, materials made of high viscosity cellulose derivatives requiring in general rather higher temperatures than materials made of low viscosity cellulose derivatives. Furthermore, the size of the inlet and outlet orifices may have an influence upon the optimum temperature for any particular degree and rate of stretching. As previously indicated, the inlet and outlet orifices are sufficiently small to enable the pressure to be maintained. Their size may be varied with the denier of the threads undergoing stretching. In general, the temperature is preferably adjusted to enable as low a stretching tension as possible to be used.

The stretched materials may be subjected to any desired after-treatment processes. Thus, the filaments, threads and other materials may be treated with shrinking agents to improve their extensibility. Suitable processes for this purpose are described in U. S. Patent No. 2,058,422. In particular reference is made to the latent solvents referred to in that specification, for example a mixture of methylene chloride and benzene.

Again, stretched cellulose ester materials may be subjected to processes of saponification. The saponification may be such as to lead to a relatively small loss in weight, for example sufficient to give the materials an affinity for cotton dye-stuffs, or may be complete or substantially complete, i. e. so as to eliminate all or substantially all of the ester content. The saponification may be effected under such conditions of tension that shrinkage takes place during or immediately after the saponification, this being advantageous from the point of view of the extensibility of the products.

Such further treatments may be carried out as operations separate from the stretching or may be carried out continuously with stretching. Thus, for example, the invention includes a continuous operation which involves first stretching and then shrinking, for example a stretching to several hundreds per cent. of the original length of the material followed by a shrinking by 7-12% of the length of the stretched material; a continuous operation involving stretching followed by saponification; and a continuous operation involving stretching, shrinking, and finally saponification.

While the invention has been described above more particularly with reference to cellulose acetate, it may also be applied to materials containing other cellulose esters or ethers, for example cellulose formate, cellulose propionate, cellulose butyrate, methyl, ethyl, or benzyl cellulose, or mixtures of esters and/or ethers or of mixed esters, ethers, or ether-esters. Furthermore, ribbons, foils, films, sheets and the like may be stretched by the processes described, and in the case of foils, films and the like the stretching may be either longitudinal and/or lateral or a lateral tension may be applied sufficient to prevent lateral shrinkage during the application of a longitudinal stretch.

Having described our invention what we desire to secure by Letters Patent is:—

1. Process for improving the strength of filaments, threads and similar textile materials and of foils, films and the like made of an organic substitution derivative of cellulose, which comprises stretching the materials in hot water under pressure at a temperature above 100° C.

2. Process for the production of lustrous filaments, threads and similar textile materials and of foils, films and the like made of an organic substitution derivative of cellulose, which materials have an improved tenacity, which comprises stretching the materials to a degree greater than the dry extensibility thereof in hot water under pressure at a temperature between 100° and 110° C. during their travel from one point to another. 45

3. Process for improving the strength of filaments, threads and similar textile materials and of foils, films and the like made of cellulose acetate, which comprises stretching the materials to a degree greater than the dry extensibility thereof in hot water under pressure at a temperature between 100° C. and 110° C. during their travel from one point to another. 50

4. Process for improving the strength of filaments, threads and similar textile materials and of foils, films and the like made of an organic substitution derivative of cellulose, which comprises stretching the materials to a degree greater than the dry extensibility thereof in hot water under pressure at a temperature of 110 to 125° C. during their travel from one point to another. 55

5. Process for improving the strength of filaments, threads and similar textile materials and of foils, films and the like made of cellulose acetate, which comprises stretching the materials to a degree greater than the dry extensibility thereof in hot water under pressure at a temperature of 110 to 125° C. during their travel from one point to another. 65

6. Process for improving the strength of filaments, threads and similar textile materials and of foils, films and the like made of an organic substitution derivative of cellulose, which comprises stretching the materials in hot water under pressure at a temperature above 125° C. 75

7. Process for improving the strength of filaments, threads and similar textile materials and of foils, films and the like made of cellulose acetate, which comprises stretching the materials to a degree greater than the dry extensibility thereof in hot water under pressure at a temperature above 125° C. during their travel from one point to another.

8. Process for improving the strength of filaments, threads and similar textile materials made of cellulose acetate, which comprises stretching the materials to at least 200% of their original length during the course of their travel through hot water under pressure at a temperature of

15 110 to 125° C.

9. Process for improving the strength of fila-

ments, threads and similar textile materials made of cellulose acetate, which comprises stretching the materials to at least 200% of their original length during the course of their travel through hot water under pressure at a temperature above 125° C. 5

10. Process for improving the strength of filaments, threads and similar textile materials made of an organic substitution derivative of cellulose, which comprises stretching the materials to at least 200% of their original length during the course of their travel through hot water under pressure at a temperature above 125° C. 10

HENRY DREYFUS.  
DONALD FINLAYSON.

15